



US008911522B2

(12) **United States Patent**  
**Cleboski et al.**

(10) **Patent No.:** **US 8,911,522 B2**  
(45) **Date of Patent:** **Dec. 16, 2014**

(54) **METHODS OF FORMING INSERTS AND EARTH-BORING TOOLS**

(75) Inventors: **Christopher J. Cleboski**, Houston, TX (US); **Suresh G. Patel**, The Woodlands, TX (US); **Danny E. Scott**, Montgomery, TX (US); **L. Allen Sinor**, Conroe, TX (US)

(73) Assignee: **Baker Hughes Incorporated**, Houston, TX (US)

(\*) Notice: Subject to any disclaimer, the term of this patent is extended or adjusted under 35 U.S.C. 154(b) by 490 days.

(21) Appl. No.: **13/176,363**

(22) Filed: **Jul. 5, 2011**

(65) **Prior Publication Data**

US 2012/0005966 A1 Jan. 12, 2012

**Related U.S. Application Data**

(60) Provisional application No. 61/361,728, filed on Jul. 6, 2010.

(51) **Int. Cl.**

*B24D 3/00* (2006.01)  
*B24B 1/00* (2006.01)  
*B24D 18/00* (2006.01)  
*C09K 3/14* (2006.01)  
*B24D 11/00* (2006.01)  
*B24D 3/02* (2006.01)  
*C09C 1/68* (2006.01)  
*E21B 10/46* (2006.01)  
*B24D 99/00* (2010.01)

(52) **U.S. Cl.**

CPC ..... *E21B 10/46* (2013.01); *B24D 99/005* (2013.01)

USPC ..... **51/295**; 51/293; 51/307

(58) **Field of Classification Search**

USPC ..... 51/295, 293, 307

See application file for complete search history.

(56) **References Cited**

U.S. PATENT DOCUMENTS

2,371,489 A 3/1945 Williams, Jr.  
3,316,073 A 4/1967 Kelso

(Continued)

FOREIGN PATENT DOCUMENTS

EP 0012631 A1 6/1980  
EP 1297928 A1 4/2003  
GB 1014295 A 12/1965

OTHER PUBLICATIONS

International Search Report for International Application No. PCT/US2011/042952 mailed Dec. 26, 2011, 4 pages.

(Continued)

*Primary Examiner* — James McDonough

(74) *Attorney, Agent, or Firm* — TraskBritt

(57) **ABSTRACT**

Methods of forming inserts for earth-boring tools include providing a material in a pattern adjacent a strip, arranging a plurality of superabrasive particles proximate the pattern, and securing at least some of the plurality of superabrasive particles to the strip. The material is configured to attract or secure the plurality of superabrasive particles. Some methods may include imparting like charges to each of a plurality of superabrasive particles, placing the plurality of superabrasive particles over a strip, and securing the superabrasive particles to the strip. In some methods, a first plurality of superabrasive particles may be placed in an array between a first strip and a second strip. A second plurality of superabrasive particles may be placed in an array between the second strip and a third strip. Methods of forming earth-boring rotary drill bits include forming an insert and securing the insert to a body of the bit.

**17 Claims, 13 Drawing Sheets**



| (56)                                                                                                                               | References Cited |                    |                  |                                   |
|------------------------------------------------------------------------------------------------------------------------------------|------------------|--------------------|------------------|-----------------------------------|
| U.S. PATENT DOCUMENTS                                                                                                              |                  |                    |                  |                                   |
| 4,574,004 A                                                                                                                        | 3/1986           | Schmidt-Ott et al. | 6,742,611 B1     | 6/2004 Illerhaus et al.           |
| 4,719,979 A                                                                                                                        | 1/1988           | Jones              | 6,843,333 B2     | 1/2005 Richert et al.             |
| 4,726,718 A                                                                                                                        | 2/1988           | Meskin et al.      | 7,350,599 B2     | 4/2008 Lockwood et al.            |
| 4,770,907 A                                                                                                                        | 9/1988           | Kimura             | 7,497,280 B2     | 3/2009 Brackin et al.             |
| 4,913,247 A                                                                                                                        | 4/1990           | Jones              | 7,776,256 B2     | 8/2010 Smith et al.               |
| 4,917,917 A                                                                                                                        | 4/1990           | Yamamoto et al.    | 7,802,495 B2     | 9/2010 Oxford et al.              |
| 4,943,488 A                                                                                                                        | 7/1990           | Sung et al.        | 2002/0194955 A1  | 12/2002 Fang et al.               |
| 5,011,514 A                                                                                                                        | 4/1991           | Cho et al.         | 2003/0084894 A1  | 5/2003 Sung                       |
| 5,025,873 A                                                                                                                        | 6/1991           | Cerkovnik          | 2004/0112359 A1* | 6/2004 Sung ..... 125/15          |
| 5,049,164 A                                                                                                                        | 9/1991           | Horton et al.      | 2004/0154840 A1  | 8/2004 Azar et al.                |
| 5,062,865 A                                                                                                                        | 11/1991          | Chen et al.        | 2004/0235406 A1  | 11/2004 Duescher                  |
| 5,096,465 A                                                                                                                        | 3/1992           | Chen et al.        | 2005/0025973 A1* | 2/2005 Slutz et al. ..... 428/408 |
| 5,143,523 A                                                                                                                        | 9/1992           | Matarrese          | 2006/0081402 A1  | 4/2006 Lockwood et al.            |
| 5,147,001 A                                                                                                                        | 9/1992           | Chow et al.        | 2007/0102198 A1  | 5/2007 Oxford et al.              |
| 5,151,107 A                                                                                                                        | 9/1992           | Cho et al.         | 2007/0102199 A1  | 5/2007 Smith et al.               |
| 5,405,573 A                                                                                                                        | 4/1995           | Clark et al.       | 2008/0202821 A1  | 8/2008 McClain et al.             |
| 6,102,140 A                                                                                                                        | 8/2000           | Boyce et al.       | 2008/0282618 A1  | 11/2008 Lockwood                  |
| 6,170,583 B1                                                                                                                       | 1/2001           | Boyce              | 2010/0122853 A1  | 5/2010 Scott et al.               |
| 6,171,709 B1                                                                                                                       | 1/2001           | Koizumi et al.     | 2010/0187011 A1  | 7/2010 Jurica et al.              |
| 6,238,280 B1                                                                                                                       | 5/2001           | Ritt et al.        | 2010/0230174 A1  | 9/2010 Scott et al.               |
| 6,286,498 B1                                                                                                                       | 9/2001           | Sung               |                  |                                   |
| 6,394,202 B2                                                                                                                       | 5/2002           | Truax et al.       |                  |                                   |
| 6,454,027 B1                                                                                                                       | 9/2002           | Fang et al.        |                  |                                   |
| 6,537,140 B1                                                                                                                       | 3/2003           | Miller et al.      |                  |                                   |
| 6,655,481 B2                                                                                                                       | 12/2003          | Findley et al.     |                  |                                   |
| OTHER PUBLICATIONS                                                                                                                 |                  |                    |                  |                                   |
| International Written Opinion for International Application No. PCT/US2011/042952 mailed Dec. 26, 2011, 4 pages.                   |                  |                    |                  |                                   |
| International Preliminary Report on Patentability for International Application No. PCT/US2011/042952 dated Jan. 8, 2013, 5 pages. |                  |                    |                  |                                   |

\* cited by examiner

**FIG. 1**

**FIG. 2**



***FIG. 3***



FIG. 4A



FIG. 4B



FIG. 4C



FIG. 4D



FIG. 4E

**FIG. 5A****FIG. 5B****FIG. 5C****FIG. 5D**





**FIG. 6A**



**FIG. 6B**



**FIG. 6C**



**FIG. 6D**



**FIG. 7A**



**FIG. 7B**



**FIG. 8A**



**FIG. 8B**



**FIG. 8C**



**FIG. 9A**



**FIG. 9B**



**FIG. 9C**



**FIG. 9D**



***FIG. 10***



**FIG. 11A**



**FIG. 11B**

**FIG. 11C**

## 1

## METHODS OF FORMING INSERTS AND EARTH-BORING TOOLS

## CROSS-REFERENCE TO RELATED APPLICATION

This application claims the benefit of U.S. Provisional Patent Application Ser. No. 61/361,728, filed Jul. 6, 2010 and entitled "Earth-Boring Tools and Intermediate Structures Formed During Fabrication Thereof Having a Controlled Distribution of Superabrasive Particles and Methods of Forming the Same," the disclosure of which is incorporated herein in its entirety by this reference.

## FIELD

Embodiments of the present disclosure relate generally to earth-boring tools for drilling subterranean formations such as drill bits, and to methods of forming such earth-boring tools.

## BACKGROUND

Wellbores are formed in subterranean formations for various purposes including, for example, the extraction of oil and gas from a subterranean formation and the extraction of geothermal heat from a subterranean formation. A wellbore may be formed in a subterranean formation using a drill bit, such as, an earth-boring rotary drill bit. Different types of earth-boring rotary drill bits are known in the art, including, for example, fixed-cutter bits (which are often referred to in the art as "drag" bits), rolling-cutter bits (which are often referred to in the art as "rock" bits), impregnated bits (impregnated with diamonds or other superabrasive superabrasive particles), and hybrid bits (which may include, for example, both fixed cutters and rolling cutters).

An earth-boring drill bit is typically mounted on the lower end of a drill string and is rotated by rotating the drill string at the surface or by actuation of downhole motors or turbines, or by both methods. The drill string may comprise a series of elongated tubular segments connected end-to-end that extends into the wellbore from the surface of the formation. When weight is applied to the drill string and consequently to the drill bit, the rotating bit engages the formation and proceeds to form a wellbore. The weight used to push the drill bit into and against the formation is often referred to as the "weight-on-bit" (WOB). As the drill bit rotates, the cutters or abrasive structures thereof cut, crush, shear, and/or abrade away the formation material to form the wellbore. A diameter of the wellbore farmed by the drill bit may be defined by the cutting structures disposed at the largest outer diameter of the drill bit.

Different types of bits work more efficiently against formations having different hardnesses. For example, bits containing inserts that are designed to shear the formation, such as fixed-cutter bits, frequently drill formations that range from soft to medium hard. These inserts often have polycrystalline diamond compacts (PDCs) as their cutting faces.

Roller cone bits are efficient and effective for drilling through formation materials that are of medium to high hardness. The mechanism for drilling with a roller cone bit is primarily a crushing and gouging action, in which the inserts of the rotating cones are impacted against the formation material. This action compresses the material beyond its compressive strength and allows the bit to cut through the formation.

For still harder formation materials, the mechanism commonly used for drilling changes from shearing to abrasion.

## 2

For abrasive drilling, bits having fixed, abrasive elements are preferred, such as diamond-impregnated bits. While bits having abrasive polycrystalline diamond cutting elements are known to be effective in some formations, they have been found to be less effective for hard, very abrasive formations. For these types of formations, cutting structures that comprise particulate diamond, or diamond grit, impregnated in a supporting matrix are generally more effective.

During abrasive drilling with a diamond-impregnated bit, 10 diamonds or other superabrasive particles scour or abrade away concentric grooves while the rock formation adjacent to the grooves is fractured and removed. Conventional impregnated drill bits typically employ a cutting face composed of superabrasive cutting particles, such as natural or synthetic diamond grit, randomly dispersed within a matrix of wear-resistant material. These diamond particles may be cast integrally with the body of the bit, as by low-pressure infiltration, or may be preformed separately, as by a hot isostatic pressure (HIP) process, to form so-called "segments" which are 15 attached to the bit by brazing or furnace to the bit body during manufacturing thereof by an infiltration process.

Diamond-impregnated bits may be formed by any one of a number of powder metallurgy processes known in the art. During the powder metallurgy process, abrasive particles 25 (e.g., diamond) and a matrix powder (e.g., tungsten carbide (WC) powder) are placed in a desired location in a mold cavity proximate a wall thereof and infiltrated with a molten binder material (e.g., a copper alloy). Upon cooling, the bit body includes the binder material, matrix material, and the 30 abrasive particles suspended both near and on the surface of the drill bit. The abrasive particles typically include small particles of natural or synthetic diamond. Synthetic diamond used in diamond impregnated drill bits is typically in the form of single crystals. However, thermally stable polycrystalline diamond (TSP) elements may also be used.

With respect to the diamond-impregnated material to be incorporated in the bit, diamond granules are formed by mixing diamonds with matrix powder and binder into a paste. The 35 paste is then packed into the desired areas of a mold. The resultant diamond-impregnated portions of the bit often have irregular diamond distribution, with areas having a cluster of too many diamonds and other areas having a lower diamond concentration, or even a void—an area free of diamonds. The diamond clusters may lack sufficient matrix material around them for good diamond retention. The areas devoid of, or low in, diamond concentration may have poor wear properties. Accordingly, bits with uncontrolled diamond distributions may fail prematurely due to uneven wear or fracturing.

Previous attempts to solve the problem of uncontrolled 40 diamond distribution include encapsulating individual diamond granules in a metal matrix material to form particles, each with a diamond granule in the center and an outer shell of metal. Then the encapsulated diamonds are mixed with a powder metal matrix and binder to form the paste, as 45 described above. One example of a similar approach is found in U.S. Pat. No. 7,350,599 to Lockwood et al., issued Apr. 1, 2008. In this way, the individual diamond granules are less likely to touch each other or cluster together and are more evenly distributed throughout the resulting paste and diamond-impregnated portions of the drill bit.

## BRIEF SUMMARY

In some embodiments, the disclosure includes a method of 55 forming an insert for an earth-boring tool comprising providing a material in a pattern adjacent a strip, arranging a plurality of superabrasive particles proximate the pattern, and

securing at least some of the plurality of superabrasive particles to the strip. The material is configured to attract or secure the plurality of superabrasive particles.

A method of forming an insert for an earth-boring tool may comprise imparting like charges to each of a plurality of superabrasive particles, placing the plurality of superabrasive particles over a strip, and securing the superabrasive particles to the strip.

In certain embodiments, a method of forming an insert for an earth-boring tool comprises placing a first plurality of superabrasive particles in an array over a first strip, placing a second strip over the first plurality of superabrasive particles, placing a second plurality of superabrasive particles in an array over the second strip, and placing a third strip over the second plurality of superabrasive particles.

Methods of forming earth-boring rotary drill bits comprise forming an insert and securing the insert to a body of the earth-boring rotary drill bit. Forming an insert comprises forming a material in a pattern over a strip, arranging the plurality of superabrasive particles proximate the pattern, and securing at least some of the plurality of superabrasive particles to the strip. The material in the pattern is configured to attract or secure a plurality of superabrasive particles.

#### BRIEF DESCRIPTION OF THE DRAWINGS

FIG. 1 is a perspective view of an embodiment of an impregnated drill bit according to the present disclosure;

FIG. 2 is a perspective view of an embodiment of a fixed-cutter drill bit according to the present disclosure;

FIG. 3 is a perspective view of a matrix-based strip prepared to receive superabrasive particles in a manner according to the present disclosure;

FIG. 4A is a perspective view of a screen for controlling the distribution of superabrasive particles on the strip of FIG. 3;

FIGS. 4B through 4E are plan views of various embodiments of the screen of FIG. 4A, detailing a portion of the screen marked by the dotted lines in FIG. 4A;

FIGS. 5A through 5F are schematic side views detailing embodiments of a process of controllably distributing superabrasive particles through the screen of FIG. 4A onto the strip of FIG. 3 according to the present disclosure;

FIGS. 6A through 6D are perspective views detailing embodiments of a process of controllably distributing superabrasive particles in recesses in the strip of FIG. 3 according to the present disclosure;

FIGS. 7A and 7B are schematic side views detailing embodiments of a process of controllably distributing superabrasive particles with an adhesive onto the strip of FIG. 3 according to the present disclosure;

FIGS. 8A through 8C are schematic views of a method of preparing superabrasive particles for electrically charging according to some embodiments of the present disclosure;

FIGS. 9A through 9D are schematic views of one embodiment of a process of controllably distributing the charged superabrasive particles of FIG. 8C onto the strip of FIG. 3 according to the present disclosure;

FIG. 10 is a schematic view of one embodiment of a process of controllably distributing the charged superabrasive particles of FIG. 8C onto the strip of FIG. 3 according to the present disclosure; and

FIGS. 11A through 11C are schematic side views of a method of using the strips prepared with superabrasive particles in a predetermined pattern, as shown in FIGS. 5D, 6D, 7B, or 9D, to form a drill bit such as those in FIG. 1 or 2.

#### DETAILED DESCRIPTION

The illustrations presented herein are not meant to be actual views of any particular material, apparatus, system, or

method, but are merely idealized representations which are employed to describe certain embodiments of the present disclosure. For clarity in description, various features and elements common among the embodiments of the disclosure may be referenced with the same or similar reference numerals.

As used herein, the term “superabrasive particles” refers to any particles having a Vickers Hardness of at least about 1000 (i.e., at least about 1200HV30, as measured according to 10 ASTM Standard E384 (Standard Test Method for Knoop and Vickers Hardness of Materials, ASTM Int’l, West Conshohocken, Pa., 2010)). Superabrasive particles may include diamond (including thermally stable polycrystalline diamond particles (TSP)), cubic boron nitride (CBN), a combination of diamond and CBN, or any other particles that have similar material hardness. The superabrasive particles may be natural or synthetic, and may be single-crystal particles or polycrystalline particles. Furthermore, the term “superabrasive particles” may refer to particles in a coated or non-coated state (e.g., in an encapsulated or non-encapsulated state). Encapsulated particles may be foliated by such methods as described in as described in Multilayer Coated Abrasive Element for Bonding to a Backing, U.S. Pat. No. 5,049,164, 15 issued Sep. 17, 1991; Low Pressure Bonding of PCD Bodies and Method for Drill Bits and the Like, U.S. Pat. No. 4,943, 20 488, issued Jul. 24, 1990; Encapsulated Diamond Particles, Materials and Impregnated Diamond Earth-Boring Bits Including Such Particles, and Methods of Forming Such Particles, Materials, and Bits, U.S. patent application Ser. No. 12/274,600, filed Nov. 8, 2008, now U.S. Pat. No. 8,069,936, 25 issued Dec. 6, 2011; and Impregnated Bit with Improved Grit Protrusion, U.S. patent application Ser. No. 12/403,734, filed Mar. 13, 2009, now U.S. Pat. No. 8,220,567, issued Jul. 17, 30 2012, the disclosures each of which are incorporated herein in their entirety by this reference. Coating materials may include, for example, tungsten, tungsten carbide, titanium, 35 titanium carbide, silicon carbide, etc.

The term “impregnated bit,” as used herein, refers to any 40 drill bit that includes superabrasive particles on or in at least one surface or bit body of the drill bit, including, for example, fixed-cutter bits, roller cone bits, and diamond-impregnated bits. While the embodiments described herein are earth-boring rotary drill bits, other drill bits, such as percussion bits, are 45 also contemplated by this disclosure. Other types of earth-boring tools, such as reamers, mills, eccentric bits, coring bits, etc., also may embody the present disclosure.

As used herein, the term “distal” refers to the side or end of the drill bit assembly that is furthest from the surface of the 50 formation that is to be drilled during normal operation.

The term “proximal,” as used herein, refers to the direction of the drill bit assembly that is closest to the surface of the formation that is to be drilled during normal operation.

The term “strip,” as used herein, refers to a body of any 55 shape and size configured to receive superabrasive particles for use in an earth-boring tool. The strips described herein may be thick or thin, wide or narrow, curved or flat, or any other combination of geometries useful for the final application. The strips described herein may be pliable or rigid.

As used herein, “ASTM mesh particles” means particles 60 that pass through an ASTM (American Society for Testing and Materials) mesh screen of a particular size as defined in ASTM specification E11-09, entitled “Standard Specification for Wire Cloth and Sieves for Testing Purposes,” which is 65 incorporated herein in its entirety by this reference. For example, a “+400 ASTM mesh particle” is a particle that is retained on, and does not pass through, an ASTM No. 400

mesh screen. A “-400 ASTM mesh particle” is a particle that does pass through an ASTM No. 400 mesh screen.

Referring to FIG. 1, according to one embodiment of the disclosure, an impregnated bit 11 may include a shank 13 of steel with threads 15 formed on its distal end for attachment to a drill string. A diamond-impregnated crown 17 is formed on the proximal end of the shank 13 (i.e., opposite threads 15). The crown 17 may have a variety of configurations. By way of example and not limitation, the crown 17 may have a plurality of blades 19 formed therein, each blade extending along the cylindrical side of the crown 17 and over to a central inverted cone area on the distal end of the crown 17. Blades 19 are separated from each other by junk slots or channels 21 for drilling fluid and cuttings return flow. In the embodiment of FIG. 1, the portion of the blades 19 on the distal end of the crown 17 are divided into segments or posts 23. Alternatively, the crown 17 may have smooth, continuous blades 19 extending to a central nozzle area. The blades 19 and posts 23 may be impregnated with diamonds or other superabrasive particles 71, as described in further detail below, to improve their performance.

While an impregnated bit 11 used for abrasive drilling is shown in FIG. 1, the disclosure contemplates other embodiments including, for example, fixed-cutter bits and rolling-cutter bits with portions or surfaces including superabrasive particles. By way of example, FIG. 2 shows a fixed-cutter bit 31 according to one embodiment that includes superabrasive particles 71 impregnated in at least one surface (e.g., a gage surface) of the fixed-cutter bit 31. Similar to the impregnated bit 11 described above, the fixed-cutter bit 31 may include a shank 33 of steel with threads 35 formed on its distal end for attachment to a drill string. A fixed-cutter crown 37 is formed on the proximal end of the shank 33 opposite the threads 35. The crown 37 may have a plurality of blades 39 formed therein separated from each other by junk slots or channels 41 for drilling fluid and cuttings return flow. The fixed-cutter bit 31 may also include cutter pockets 42 in the blades 39 configured to receive cutting elements 44. The cutter pockets 42 may include buttresses 43 to support the cutting elements 44 from the rear. Cutting elements 44 may have a face made of polycrystalline diamond compact (PDC) or some other hard material for shearing away the formation to be drilled.

The fixed-cutter bit 31 shown in FIG. 2 may also include a structure referred to as a bit gage 45, defined by gage pads 46. The bit gage 45 may be positioned at the base of blades 39 such that the surface of the bit gage 45 is at the largest diameter of the fixed-cutter bit 31. Therefore, as the fixed-cutter bit 31 rotates and drills through the formation, the bit gage 45 may be engaged with the formation on the walls of the hole that is formed as the fixed-cutter bit 31 drills through the formation. The gage pads 46 may be provided at the bit gage 45 to decrease wear of the base of the blades 39 and to ensure that diameter of the fixed-cutter bit 31 and the resulting diameter of the hole in the formation stay substantially constant as drilling progresses. Therefore, the gage pads 46 may include superabrasive particles 71 and may be formed from superabrasive particle-impregnated strips 91 that will be described in more detail hereinafter.

An embodiment of a process and system for arranging superabrasive particles 71 in a predetermined pattern and controlled manner will now be described. In short, the method includes providing a material in a pattern over a strip, arranging particles proximate the pattern, and securing the particles to the strip. As shown in FIG. 3, a strip 61 (e.g., a matrix-based strip, a paper, a polymer, etc.) may be prepared to receive diamonds or other superabrasive particles 71. Although the strip 61 is shown as a generally flat rectangular material, the

strip 61 may have any desired shape or size. For example, in some embodiments, the strip 61 may have an irregular shape to match the feature of the impregnated bit 11 that is to be formed from the strip 61. In other embodiments, the strip 61 may be circular, semicircular, triangular, trapezoidal, etc. The strip 61 may have a major surface that is flat, curved, stepped, or any combination thereof. In addition, the strip 61 may have a generic shape, such as rectangular, that is later shaped by trimming, cold pressing, bending, etc. In other words, the strip 61 may have any shape or size that is convenient for the final application, as will be appreciated by one of ordinary skill in the art.

In some embodiments, it may be advantageous for the strip 61 to comprise a matrix material therein, as discussed in further detail below, that, upon further processing (e.g., infiltration or sintering), will have a sufficient hardness so that superabrasive particles 71 exposed at the cutting face are not pushed further into the matrix material under the high pressures used in drilling. In addition, the matrix may have sufficient bond strength with the superabrasive particles 71 so that the superabrasive particles are not prematurely released. Finally, the heating and cooling time during subsequent sintering, hot-pressing, or infiltration, as well as the maximum temperature of the thermal cycle, may be sufficiently low so that the superabrasive particles embedded in the strip 61 are not thermally damaged during the process.

Therefore, in some exemplary embodiments, the strip 61 may include hard particles 63, which may or may not be characterized as superabrasive particles, bound together by, for example, an organic binder 62. The hard particles 63 may comprise diamond or hard and abrasion resistant ceramic materials such as carbides, nitrides (including cubic boron nitride, or CBN), oxides, and borides (including boron carbide (B<sub>4</sub>C)). More specifically, the hard particles 63 may comprise carbides and borides made from elements such as W, Ti, Mo, Nb, V, Hf, Ta, Cr, Al, or Si. By way of example and not limitation, materials that may be used to form the hard particles 63 include tungsten carbide (WC or W<sub>2</sub>C, including macrocrystalline tungsten carbide and cemented or sintered tungsten carbide), titanium carbide (TiC), tantalum carbide (TaC), titanium diboride (TiB<sub>2</sub>), chromium carbides, titanium nitride (TiN), vanadium carbide (VC), aluminum oxide (Al<sub>2</sub>O<sub>3</sub>), aluminum nitride (AlN), boron nitride (BN), and silicon carbide (SiC). The strip may be formed by, for example, cold pressing the hard particles 63 and the organic binder 62.

Combinations of different hard particles may be used to tailor the physical properties and characteristics of the particle-matrix composite material of the portion of the drill bit to be impregnated with superabrasive particles 71. For example, alloys and mixtures may also be used, including tungsten alloys such as tungsten/cobalt (W/Co) alloys, tungsten carbide (WC or W<sub>2</sub>C) or tungsten carbide/cobalt (WC/Co or W<sub>2</sub>C/Co) alloys in combination with elemental tungsten (e.g., with an appropriate binder phase to facilitate bonding of particles and diamonds). The hard particles 63 may be formed using techniques known to those of ordinary skill in the art. In some embodiments, tougher materials may be applied before harder, more wear resistant particles. For example, tungsten carbide particles may be disposed in a strip 61 under diamond particles for tools intended to drill through steel (e.g., casing) or iron rich formations. Particles may be configured as described in Cutting Structures For Casing Component Drillout And Earth-Boring Drill Bits Including Same, U.S. patent application Ser. No. 12/604,899, filed Oct.

23, 2009, now U.S. Pat. No. 8,245,797, issued Aug. 21, 2012, the disclosure of which is incorporated herein in its entirety by this reference.

The binder 62 of the strip 61, shown in FIG. 3, may, in some embodiments, be or include an organic binder. Examples of organic binders include polyethylene, polyethylene-butyl acetate (PEBA), ethylene vinyl acetate (EVA), ethylene ethyl acetate, polyethylene glycol (PEG), polypropylene (PP), poly vinyl alcohol (PVA), polystyrene (PS), polymethyl methacrylate, poly ethylene carbonate (PEC), polyalkylene carbonate (PAC), polycarbonate, poly propylene carbonate (PPC), nylons, polyvinyl chlorides, polybutenes, polyesters, etc. In other embodiments, the binder 62 can include, for example, aqueous and gelation polymers or inorganic polymers. Suitable aqueous and gelation polymers may include those formed from cellulose, alginates, polyvinyl alcohol, polyethylene glycol, polysaccharides, water, and mixtures thereof. Silicone is an example of an inorganic polymer binder. Other binders 62 may include wax or natural and synthetic oil (e.g., mineral oil) and mixtures thereof. It is contemplated that one of ordinary skill in the art may find other binders useful for the binder 62 as deemed available and appropriate for binding the hard particles 63 together and for receiving superabrasive particles 71, in the manner described in more detail below.

Thus, in some embodiments, the strip 61 may have the consistency of a paste. In other embodiments, the strip 61 may have the consistency of a flexible elastomer, or of a relatively rigid thermoplastic material. The strip 61 may nevertheless be quite soft when compared to the hardness of the superabrasive particles.

In some embodiments, the strip 61 may comprise a powdered binder material, formed by cold pressing. In other embodiments, the strip 61 may be a thin flexible material, such as paper. The strip 61 with superabrasive particles 71 may be flexible, such that it may conform to surfaces, such as surfaces of molds for forming earth-boring tools.

A material configured to attract or secure superabrasive particles may be provided in a pattern adjacent the strip 61. For example, a template having a plurality of apertures may be placed over the strip 61. A screen 51, as shown in FIGS. 4A through 4E, may be positioned over at least one surface of the strip 61 for arranging diamonds or other superabrasive particles 71 according to a predetermined pattern and in a controlled fashion on and/or in the strip 61. Although FIG. 4A shows the screen 51 in a generally flat rectangular shape, the screen 51 may be any desired shape, including, for example, flat or curved, circular, triangular, trapezoidal, irregular, etc. The shape of the screen 51 may be determined by the shape of an area of an impregnated bit 11, for example, which is to have superabrasive particles 71 distributed in a controlled manner. In other embodiments, it may be desirable for screen 51 to have an overall shape that is larger than the corresponding shape of the strip 61 to be impregnated with superabrasive particles 71, to ensure full coverage of the strip 61 with superabrasive particles 71 arranged in a predetermined pattern.

As can be seen in FIGS. 4B through 4E, the screen 51 may be fowled from a variety of materials and in a variety of configurations. The screen 51 may comprise any of a number of suitable materials, including, for example, polymer materials, metal materials, ceramic materials, and combinations of such materials. The screen 51 may have any of a number of configurations, such as those shown in FIGS. 4B through 4E as 51b through 51e. For example, in one embodiment, the screen 51b may be formed with wires or threads 52 woven or overlapping to form a grid structure, as shown in FIG. 4B. In this embodiment, apertures 54 for receiving and allowing

passage of superabrasive particles 71 therethrough may extend through the screen 51 and between the wires or threads 52. In other embodiments, shown in FIGS. 4C through 4E, the screen 51c through 51e may comprise a sheet 53 and a plurality of apertures 54 extending through the sheet 53. The sheet 53 may comprise one or more layers of any of the materials mentioned above. The apertures 54 may be formed in the sheet 53 by various methods. For example, the apertures 54 may be formed by laser ablation, stamping, drilling, cutting, masking and etching, and/or any other suitable method for creating apertures 54 in the sheets 53. In other embodiments, the apertures 54 may be formed during fabrication of the sheets 53, such that no additional processing is needed to form the apertures 54 through the sheets 53 after fabrication of the sheets 53. As shown by way of example in FIG. 4C, the apertures 54 in the screen 51c may be generally square in shape. In additional embodiments, as shown in FIGS. 4D and 4E, the apertures 54 may be circular. It is contemplated that the shape of the apertures 54 may be any desired shape, including square, rectangular, triangular, circular, irregular, etc.

Referring again to the embodiment of the screen 51c shown in FIG. 4C, the plurality of apertures 54 may be arranged in a rectangular grid pattern, such that the apertures 54 are arranged in discrete rows and columns on the sheet 53. However, in other embodiments, such as that shown in FIG. 4D, the apertures 54 in the screen 51d may be arranged at an angle to each other, or, in other words, the apertures 54 in one row may be staggered or shifted in position relative to one or more adjacent rows. Such configurations may allow the superabrasive particles 71 to be positioned in a closer packed arrangement than configurations in which the apertures are arranged in rows and columns, such as shown in FIG. 4C.

In another embodiment shown in FIG. 4E, the apertures 54 may be arranged in an irregular fashion, with a higher concentration of apertures 54 through the sheet 53 in one or more locations on the screen 51e, and a lower concentration of apertures 54 through the sheet 53 in other locations on the screen 51e. In this manner, the superabrasive particles 71 that will be placed on the strip 61 through the screen 51e may be concentrated on the strip 61 as desired, such as, for example, at the leading edge of a blade 19 or post 23.

The apertures 54 shown in FIGS. 4B through 4E may be sized as desired to receive one or more superabrasive particles 71 through each aperture 54. The size and shape of each aperture 54 can be tailored to match or exceed, for example, the mesh size of the superabrasive particles 71. The mesh size of the superabrasive particles 71 may be, for example, from +20 ASTM (American Society for Testing and Materials) to -400 ASTM, or approximately 37 microns to 841 microns in diameter. More specifically, the superabrasive particles 71 may be -40/+50 ASTM mesh particles, or approximately 297 microns to 420 microns in diameter. Alternatively, the superabrasive particles 71 may be -25/+35 ASTM mesh particles, or approximately 500 microns to 707 microns in diameter. In certain embodiments, the mesh size may be as large as necessary to accommodate selected superabrasive particles 71. Thus, the apertures 54 in the screen 51 may be sized to receive one or more superabrasive particles 71 by matching or exceeding the mesh size of the superabrasive particles 71. In some embodiments, it may be desirable to size the apertures 54 so that only one superabrasive particle 71 will fit through each aperture 54 and onto the surface of the strip 61. In such embodiments, each aperture 54 may have a diameter that is slightly larger than the average diameter of superabrasive particles 71, but less than two times the average diameter of the superabrasive particles 71.

Once the strip 61 and screen 51 are prepared, the screen 51 may be placed over one or more surfaces of the strip 61, as shown in FIG. 5A. Superabrasive particles 71 may then be placed over the screen 51, so that at least some of the superabrasive particles 71 fall into or through the screen 51 and onto the strip 61. Thus, at least some of the superabrasive particles 71 may be placed in the pattern defined by the screen 51. To facilitate the distribution of the superabrasive particles 71 and the filling of the apertures 54, the assembly may be shaken, agitated, tilted, vibrated, pressed, blown with air, etc. Optionally, excess superabrasive particles 71 (i.e., those that have not fallen into apertures 54) may be removed by using a squeegee, scraping, tilting the assembly, blowing, or vacuuming the excess superabrasive particles 71, brushing or shaking the excess superabrasive particles 71 off, etc., resulting in the assembly shown in FIG. 5B. In some embodiments, one superabrasive particle 71 may be disposed at least partially within each aperture 54 of a plurality of apertures 54 through the screen 51. It is not necessary that each and every aperture 54 have a superabrasive particle 71 disposed therein, but it is contemplated that some of the plurality of apertures 54 will each have a superabrasive particle 71 disposed therein. In other embodiments, each and every aperture 54 may have one or more superabrasive particles 71 at least partially disposed therein.

Referring now to FIGS. 5C and 5D, the superabrasive particles 71 may be secured by pressing them into the strip 61. In one embodiment, a plate 81 is placed over the screen 51 and superabrasive particles 71. The plate 81 is pressed against the superabrasive particles 71, as shown by force arrows 83. This forces the superabrasive particles 71 at least partially into the strip 61, as shown in FIG. 5D. The screen 51 may have an average thickness that is less than the average diameter of the superabrasive particles 71. In other embodiments, the screen 51 may have an average thickness that is greater than the average diameter of the superabrasive particles 71, and a punch or rod-like device may be used to push each superabrasive particle 71 through the apertures 54 in the screen 51. For example, the plate 81 may have protrusions or pins on a lower side corresponding to locations of the apertures 54. The plate 81 may be formed of a material that is harder than the strip 61 in its preform state, such as metal, plastic, or ceramic. While FIG. 5C shows the pressing of the superabrasive particles 71 into the strip 61 with a plate 81, it is contemplated that the superabrasive particles 71 may be pressed into the plate 81 in other ways that will be apparent to one of ordinary skill in the art. For example, a roller (not shown) may roll over the surface, pressing the superabrasive particles 71 into the strip 61 as it rolls. In other embodiments, the superabrasive particles 71 may be tapped into place with a device (not shown) of suitable hardness. The screen 51 may optionally be removed prior to or after the pressing of the superabrasive particles 71 into the strip 61. In some embodiments, the screen 51 may stay in place if, for example, it is made of a material (such as a polymer) that may be burned off later in the process, or of a ceramic or metal that may be incorporated into the final product during sintering or infiltration, without significantly compromising the mechanical properties of the final product. In yet other embodiments, the superabrasive particles 71 may be partially pressed into the strip 61 with the screen 51 in place, the screen 51 may then be removed, and the superabrasive particles 71 may finally be pressed further into the strip 61 after the screen 51 is removed.

The resulting structure 91 shown in FIG. 5D may comprise a strip 61 with superabrasive particles 71 distributed in a predetermined pattern partially or fully across at least one surface of the strip 61. The superabrasive particles 71 may be

fully embedded (not shown) or partially embedded in the strip 61. This resulting structure 91 may be referred to as a soft insert 91 or green insert 91 because it has not yet been sintered, infiltrated, cured, or otherwise processed to assume its final, hard configuration.

Instead of or in addition to pressing the superabrasive particles 71 into the strip 61, the superabrasive particles may be secured by a second strip 61a, as shown in FIGS. 5E and 5F. The second strip 61a may have the same or a different composition or dimension as the strip 61. The screen 51 may or may not be removed from the strip 61 before placing the second strip 61a over the strip 61 and the superabrasive particles 71.

The superabrasive particles 71 may, in some embodiments, be secured to the strip 61 by hot isostatic pressing (HIP), a hot pressing process, an infiltration process, etc.

Using the screen 51 described above is but one method of arranging superabrasive particles over a strip 61. In other embodiments, for example as shown in FIG. 6A, a plurality of recesses 65 may be formed in a strip 61. The recesses 65 may be sized as desired to receive one or more superabrasive particles 71 within each recess 65, as shown in FIG. 6B. The size and shape of each recess 65 can be tailored to match or exceed, for example, the mesh size of the superabrasive particles 71. The mesh size of the superabrasive particles 71 may be, for example, from +20 ASTM (American Society for Testing and Materials) to -400 ASTM, or approximately 37 microns to 841 microns in diameter. More specifically, the superabrasive particles 71 may be -40/+50 ASTM mesh particles, or approximately 297 microns to 420 microns in diameter. Alternatively, the superabrasive particles 71 may be -25/+35 ASTM mesh particles, or approximately 500 microns to 707 microns in diameter. The superabrasive particles 71 may be of any selected size and shape. Thus, the recesses 65 in the strip 61 may be sized to receive one or more superabrasive particles 71 by matching or exceeding the mesh size of the superabrasive particles 71. In some embodiments, it may be desirable to size the recesses 65 so that only one superabrasive particle 71 will fit within each recess 65. In such embodiments, each recess 65 may have a diameter that is slightly larger than the average diameter of the superabrasive particles 71, but less than two times the average diameter of the superabrasive particles 71.

Superabrasive particles 71 may then be placed over the strip 61, so that at least some of the superabrasive particles 71 fall into the recesses 65. Thus, at least some of the superabrasive particles 71 may be arranged in a pattern defined by the recesses 65. To facilitate the distribution of the superabrasive particles 71 and the filling of the recesses 65, the assembly may be shaken, agitated, tilted, vibrated, pressed, blown with air, etc. Optionally, excess superabrasive particles 71 (i.e., those that have not fallen into recesses 65) may be removed by using a squeegee, scraping, tilting the assembly, blowing, or vacuuming the excess superabrasive particles 71, brushing or shaking the excess superabrasive particles 71 off, etc., resulting in the assembly shown in FIG. 6B. In some embodiments, one superabrasive particle 71 may be disposed at least partially within each recesses 65 of a plurality of recesses 65. It is not necessary that each and every recess 65 have a superabrasive particle 71 disposed therein, but it is contemplated that some of the plurality of recesses 65 will each have a superabrasive particle 71 disposed therein. In other embodiments, each and every recess 65 may have one or more superabrasive particles 71 at least partially disposed therein.

In some embodiments, the superabrasive particles 71 may be individually placed into recesses 65. For example, an SMT (surface mount technology) component placement system

## 11

(commonly referred to as a pick-and-place machine) may be used to place superabrasive particles 71 within recesses. The superabrasive particles 71 may be placed concurrently with the formation of the strip 61, such as in a single rapid-prototyping operation.

The superabrasive particles 71 disposed within the recesses 65 may then be secured to the strip 61, such as by the pressing methods previously described. For example, as shown in FIG. 6C, a second strip 61a may be disposed (e.g., placed or formed) atop the strip 61 and the superabrasive particles 71. The second strip 61a may have recesses (not visible in FIG. 6C) on a lower surface of the strip 61a arranged to align with the recesses 65 of the first strip 61. When the second strip 61a is placed over the strip 61, the recesses on the lower surface of the second strip 61a may align with recesses 65 of the first strip 61 to form enclosed cavities in which superabrasive particles 71 are confined. In some embodiments, the depth of the recesses 65 of the first strip 61 or of the second strip 61a may be less than half of the average diameter of the superabrasive particles 71, such that at least some of the superabrasive particles 71 become embedded into the first strip 61 and/or the second strip 61a when the two strips are pressed together, forming a sandwiched array of superabrasive particles. In some embodiments, the lower surface of the second strip 61a may not have recesses therein, and pressing the second strip over the superabrasive particles 71 may cause the superabrasive particles 71 to become embedded into the first strip 61 and/or the second strip 61a. The second strip 61a may have recesses 65 in an upper surface (e.g., a surface on an opposite side from the side adjacent the first strip 61) configured to accept superabrasive particles 71. The recesses 65 in the upper surface of the second strip 61a may be directly above the recesses 65 in the first strip 61, or may be staggered or offset from the recesses 65 in the first strip 61. The size, density, and location of the recesses 65 may be varied to achieve any selected arrangement of superabrasive particles 71. Additional superabrasive particles 71 may be disposed within these recesses 65, and a third strip 61b, shown in FIG. 6D, may be applied in the same manner. The superabrasive particles 71 applied over the second strip 61a may have the same or different sizes, compositions, or coatings than the superabrasive particles 71 applied between the first strip 61 and the second strip 61a. Strips and superabrasive particles 71 may be added in as many layers and configurations as necessary to form a green insert 91 having a desired arrangement of superabrasive particles 71.

The strips 61, 61a, or 61b, and/or the recesses 65 therein, may be formed by, for example, injection molding, powder metal pressing, hydraulic pressing in a mold, rapid prototyping, applying a die or a plate with protruding pins, etc. The strips 61, 61a, or 61b, and/or the recesses 65 may be formed in situ, or may be separately formed before arrangement with the superabrasive particles 71. The recesses 65 are shown in FIGS. 6A through 6C as dimples (e.g., approximately hemispherical), but may be any shape. The recesses 65 are shown in FIGS. 6A through 6C as distinct, but they may also be connected. For example, the recesses 65 may take the form of an array of connected troughs in a grid or mesh pattern. Superabrasive particles 71 may be placed within the troughs and secured as described above.

Another method of arranging superabrasive particles 71 over a strip 61 is shown in FIGS. 7A and 7B. In some embodiments, an adhesive 66 may be provided over a strip 61. The adhesive 66 may include a glue, cement, or epoxy, and may be formed in a pattern. For example, an array of glue dots may be applied on the strip 61. In some embodiments, the adhesive 66 may form a grid or mesh pattern. Superabrasive particles 71

## 12

may be disposed over the adhesive 66, such as by spreading superabrasive particles 71 over the entire strip 61. Some of the superabrasive particles 71 may be attracted to the adhesive 66 (e.g., may adhere to the adhesive), and other superabrasive particles 71 may not be attracted to the adhesive 66. As shown in FIG. 7B, excess superabrasive particles 71 (e.g., superabrasive particles 71 that are not attracted to the adhesive) may be removed from the strip 61, such as by shaking, agitating, tilting, vibrating, blowing air, vacuuming, brushing, etc. The superabrasive particles 71 may optionally be pressed into the strip 61 for additional security. Multiple strips 61 may be stacked, and may be bonded by another adhesive, a matrix material, etc. The strips 61 may be removed during processing (e.g., by burning or otherwise reacting material of the strip 61), or may ultimately become a part of an earth-boring tool.

Another method and apparatus for distributing superabrasive particles 71 on and in a strip 61 for inclusion in abrasive applications, such as earth-boring drill bits, will now be disclosed. A strip 61 may be prepared as discussed previously. Instead of using a screen 51 or recesses 65 to align the superabrasive particles 71, the superabrasive particles 71 may be electrically charged, as shown in FIGS. 8A through 8C. Superabrasive particles 71, such as diamonds or cubic boron nitride (CBN) particles, are provided, as shown in FIG. 8A and as described previously. As shown in FIG. 8B, each superabrasive particle 71 may subsequently be coated with a chargeable coating 73. The chargeable coating 73 may be a metal, such as, by way of non-limiting example, iron (Fe), copper (Cu), cobalt (Co), tungsten (W), nickel (Ni), etc. In some embodiments, a chargeable coating 73 of tungsten may provide a desirable bond with the matrix material of the strip 61 or body of the drill bit. The chargeable coating 73 may be formed on the superabrasive particles by chemical vapor deposition (CVD), or by mechanical milling (e.g., ball milling) of the diamond particles with particles of metal (e.g., tungsten metal), as will be appreciated by one of ordinary skill in the art. The chargeable coating 73 may be a thin layer, for example, approximately 5 to 10 microns in thickness around each superabrasive particle 71. The resulting particle is a coated superabrasive particle 75, as shown in FIG. 8B.

Referring to FIG. 8C, the chargeable coating 73 on the superabrasive particles 71 may be electrically charged. The electrical charging of the coated superabrasive particle 75 may be accomplished in any of a number of ways. For example, an electrostatic gun, such as a corona spray gun, may be loaded with the coated superabrasive particles 75. A corona gun produces an electrical discharge brought on by the ionization of the coated superabrasive particles 75 surrounding an electrode, which occurs when the potential gradient exceeds approximately 30 kV per centimeter. The coated superabrasive particles 75 may exit the corona gun and travel near an electrode where they accumulate an electrical charge. As another non-limiting example, a "tribo" gun may be used to charge the coated superabrasive particles 75 by friction. The coated superabrasive particles 75 may be forced or blown through a polytetrafluoroethylene (PTFE) tube and may accumulate an electric charge while rubbing along the walls of the tube. In yet another non-limiting example, the coated superabrasive particles 75 may be loaded into a metal container, and mixed with an aluminum mixing blade mounted on an insulating shaft. The outside of the metal container may be grounded to reduce the risk of capacitive electrostatic discharge from the outside of the vessel. Although the coated superabrasive particles 75 are shown in the figures with a negative electrical charge, it is to be understood that the coated superabrasive particles 75 may be electrically charged with either a negative or a positive charge. Each coated

superabrasive particle 75 may have the same charge (i.e., all charged coated superabrasive particles 75 may be positively charged or all charged coated superabrasive particles 75 may be negatively charged). Like charges on the coated superabrasive particles 75 may assist in proper dispersion of the coated superabrasive particle 75.

Referring to FIGS. 9A and 9B, a strip 61 may be prepared as described above. The strip 61 may be electrically charged with a charge opposite that of the charged coated superabrasive particles 75 (shown in FIG. 9A), or, alternatively, the strip 61 may be electrically grounded (shown in FIG. 9B). In some embodiments, it may be desirable to ensure that the strip 61 is prepared with a binder, hard particles, or further additives that are electrically conductive so that the strip 61 may hold an electrical charge. After the strip 61 is electrically charged or grounded, the charged coated superabrasive particles 75 may be placed on the charged or grounded strip 61. The opposite charging or the grounding of the strip 61 may tend to attract the charged coated superabrasive particles 75 so they stick to the surface of the strip 61 by the electrical forces involved. In some embodiments, a screen 51 or other physical object may not be necessary to evenly distribute the charged coated superabrasive particles 75 because the similar electrical charge on each coated superabrasive particle 75 will tend to repel the coated superabrasive particles 75 away from each other. In this manner, the charged coated superabrasive particles 75 may distribute themselves across the surface of the strip 61 in a way that reduces, minimizes, or prevents clustering. Agitating the assembly may facilitate the movement and even distribution of the coated superabrasive particles 75 on the surface of the strip 61.

Referring now to FIGS. 9C and 9D, after the coated superabrasive particles 75 are distributed and dispersed on the surface of the strip 61, the coated superabrasive particles 75 may be pressed into the strip 61 with a plate 81 by a force 83, as described previously. In this case, the plate 81 may be formed from an electrically insulating material or with an insulating handle so as to not conduct away the charge of the particles and/or the strip 61. After pressing, the resulting structure 91 may comprise a matrix-based strip 61 with coated superabrasive particles 75 pressed therein and distributed in a controlled manner. As in FIG. 5D, the resulting structure 91 shown in FIG. 9D may be referred to as a soft insert 91 or green insert 91.

In some embodiments shown in FIG. 10, a chargeable coating 73 over superabrasive particles 71 may be a magnetic material. Coated superabrasive particle 75 may be placed on a strip 61. A wire mesh 85 may be placed proximate an opposite side of the strip 61 from the coated superabrasive particles 75. The wire mesh 85 may be electrically charged, forming a magnetic field. The coated superabrasive particles 75 may align with a portion of the resulting magnetic field. Optionally, coated superabrasive particles 75 not aligned with the magnetic field may be removed, such as by shaking, agitating, tilting, vibrating, blowing air, vacuuming, brushing, etc. Once aligned, the coated superabrasive particles 75 may be secured into place, such as by pressing, spraying with powder coat, placing another strip 61a over the coated superabrasive particles 75, etc.

The superabrasive particles 71 may be individually placed on a strip 61. For example, an SMT component placement system may be used to place superabrasive particles 71 in precise locations on a strip 61. In some embodiments, superabrasive particles 71 may be placed by hand, such as underneath a magnifying viewer. Once aligned, the superabrasive particles 71 may be secured into place, such as by pressing,

spraying with powder coat, placing another strip 61a over the superabrasive particles 71, etc.

In some embodiments, the methods described above may be repeated and/or combined to provide more than one layer 5 of superabrasive particles 71 and one or more strips 61. For example, the process may be repeated on a different surface, such as the back or opposite surface of the strip 61. In other embodiments, more than one strip 61 may be stacked and pressed together to form a green insert 91 with multiple layers 10 of superabrasive particles 71, each distributed according to a predetermined pattern. The pattern of the superabrasive particles 71 may have uniform or varied spacing, and may be formed in a spiraled, staggered, or other pattern to produce a selected wear pattern. Combinations of different diameters of superabrasive particles 71, variation of spacing between superabrasive particles 71, different compositions and coatings of superabrasive particles 71, etc. may be used to achieve a selected wear pattern. The diameter and/or concentration of the superabrasive particles 71 (and therefore the wear pattern) may be selectively varied along dimensions of an insert for an earth-boring tool. For example, the wear pattern may be varied front-to-back, center-to-outside, top-to-bottom, or any combination thereof. The variation may be within a single strip 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055

Preheating may be conducted in a furnace or other heating device, such as an induction coil, as is known in the art.

Turning to FIG. 11C, infiltration may be conducted at typical infiltration temperatures, for example, temperatures of from about 950° C. to about 1200° C. or hotter, at which a hardenable liquid infiltrant material 107 will liquefy and will imbibe substantially throughout the various particulate-based regions of the bit body, including the inserts 91.

A conventional infiltrant material 107, such as a copper or copper-nickel alloy or a high melting-point non-metallic binder, such as a glass-based material, may be employed to infiltrate the inserts 91 and the rest of the bit body. Alternatively, a polymeric binder, such as a polyester or an epoxy resin, may be employed to infiltrate the inserts 91 and the remainder of the bit body. In some instances, infiltration with such material may be carried out at substantially room temperature.

With continued reference to FIG. 11C, a hardenable liquid infiltrant material 107 may be placed in contact with the particulate core material 105 disposed in the mold interior 104 and mass infiltrated into the interstices between particles of the core material 105 and into the interstices of the insert or inserts 91, as is known in the art. During infiltration, the infiltrant material 107 melts and moves throughout the particulate-based regions of the core material or materials 105 and of the inserts 91.

The infiltrant material 107 is then permitted to harden and solidify, effectively binding the particles comprising the impregnated bit 11 together. As the infiltrant material 107 solidifies, it may also bind the bit body to any solid structures disposed therein, such as a bit blank or bit shank (shown in FIG. 1), resulting in a single, integral structure. The infiltrant material 107 may also fill any voids within or on the bit body. The infiltrant material 107 may also infiltrate the insert or inserts 91 and, thereby, integrate the inserts 91 with the remainder of the bit body.

Alternatively, the insert or inserts 91 may be infiltrated prior to infiltrating the remainder of the bit body. The insert or inserts 91 may subsequently be secured to the remainder of the bit body during infiltration by the infiltrant material 107 bonding to the material with which the insert 91 is infiltrated. Alternatively, the insert 91 may subsequently be secured to the remainder of the bit body by, for example, mechanical means, brazing, welding, or adhering, as will be appreciated by one of ordinary skill in the art.

In other embodiments, similar methods to those described may be used to include inserts 91 with a controlled distribution of superabrasive particles 71 in fixed-cutter bits 31, such as the fixed-cutter bit 31 shown in FIG. 2.

In yet additional embodiments, the inserts 91 may be incorporated into a green bit body, such as a pressed, green bit body, which then may be sintered to form a drill bit like that shown in FIG. 1 or that shown in FIG. 2, using methods such as those disclosed in, for example, U.S. Pat. No. 7,776,256, issued Aug. 17, 2010 to Smith et al., and U.S. Patent Application Publication No. US 2007/0102198A1, which was filed Nov. 10, 2005, now U.S. Pat. No. 7,802,495, issued Sep. 28, 2010, in the name of Oxford et al., the disclosures of which are incorporated herein in their respective entireties by this reference.

Embodiments of the present disclosure, therefore, may find use in any application in which diamond-impregnated or superabrasive particle-impregnated materials may be used. Specifically, embodiments of the present disclosure may be used to create diamond impregnated inserts, diamond impregnated bit bodies, diamond impregnated wear pads, or any other diamond impregnated material known to those of

ordinary skill in the art. Further, embodiments of the present disclosure may be used in diamond impregnated cutter wheels, diamond impregnated grinding wheels, diamond impregnated saws, diamond impregnated core drills, diamond impregnated blades, etc.

Additional non-limiting example embodiments of the disclosure are described below.

Embodiment 1: A method of forming an insert for an earth-boring tool comprising providing a material in a pattern adjacent a strip, arranging a plurality of superabrasive particles proximate the pattern, and securing at least some of the plurality of superabrasive particles to the strip. The material is configured to attract or secure the plurality of superabrasive particles.

Embodiment 2: The method of Embodiment 1, wherein securing at least some of the plurality of superabrasive particles to the strip comprises pressing at least some of the plurality of superabrasive particles into the strip.

Embodiment 3: The method of Embodiment 2, wherein providing a material in a pattern over a strip comprises placing a template having a plurality of apertures over the strip, and wherein arranging a plurality of superabrasive particles proximate the pattern comprises placing at least some of the plurality of superabrasive particle at least partially within at least some of the apertures.

Embodiment 4: The method of any of Embodiments 1 through 3, further comprising infiltrating the strip with a metallic binder after arranging the plurality of superabrasive particles.

Embodiment 5: The method of any of Embodiments 1 through 4, further comprising subjecting the strip and the superabrasive particles to a hot isostatic pressing process.

Embodiment 6: The method of any of Embodiments 1 through 5, wherein providing a material in a pattern over a strip comprises forming the material to have a plurality of recesses therein, and arranging the plurality of superabrasive particles proximate the pattern comprises disposing a superabrasive particle within each recess of the plurality of recesses in the material.

Embodiment 7: The method of any of Embodiments 1 through 6, further comprising disposing another strip over the superabrasive particles and the strip to form a sandwiched array of superabrasive particles.

Embodiment 8: The method of Embodiment 7, wherein disposing another strip over the superabrasive particles and the strip to form a sandwiched array of superabrasive particles comprises embedding at least some of the plurality of superabrasive particles into at least one of the strip and the another strip.

Embodiment 9: The method of Embodiment 7, further comprising disposing a superabrasive particle within each recess of the plurality of recesses of the another strip, and forming a third strip over the another strip and the superabrasive particles.

Embodiment 10: The method of any of Embodiments 1 through 9, wherein providing a material in a pattern over a strip comprises providing adhesive on the strip. Arranging the plurality of superabrasive particles proximate the pattern comprises disposing the plurality of superabrasive particles over the strip, such that some particles of the plurality are attracted to the adhesive, and removing particles of the plurality that are not attracted to the adhesive.

Embodiment 11: The method of any of Embodiments 1 through 10, further comprising coating each superabrasive particle of the plurality of superabrasive particles with a magnetic material and disposing a charged mesh under the strip.

## 17

Embodiment 12: A method of forming an insert for an earth-boring tool, comprising, imparting like charges to each of a plurality of superabrasive particles, placing the plurality of superabrasive particles over a strip, and securing the superabrasive particles to the strip.

Embodiment 13: The method of Embodiment 12, further comprising coating each superabrasive particle of the plurality of superabrasive particles with a chargeable material.

Embodiment 14: The method of Embodiment 12 or Embodiment 13, wherein securing the superabrasive particles to the strip comprises pressing the particles at least partially into the strip.

Embodiment 15: A method of forming an insert for an earth-boring tool, comprising placing a first plurality of superabrasive particles in an array over a first strip, placing a second strip over the first plurality of superabrasive particles, placing a second plurality of superabrasive particles in an array over the second strip, and placing a third strip over the second plurality of superabrasive particles.

Embodiment 16: The method of Embodiment 15, further comprising subjecting the strips and the superabrasive particles to a hot isostatic pressing process.

Embodiment 17: A method of forming an earth-boring rotary drill bit, comprising forming an insert and securing the insert to a body of the earth-boring rotary drill bit. Forming an insert comprises forming a material in a pattern over a strip, arranging the plurality of superabrasive particles proximate the pattern, and securing at least some of the plurality of superabrasive particles to the strip. The material in the pattern is configured to attract or secure a plurality of superabrasive particles.

Embodiment 18: The method of Embodiment 17, wherein securing the insert to a body of the earth-boring rotary drill bit comprises placing the insert in a mold for an earth-boring rotary drill bit, placing particulate core materials in the mold, and infiltrating the particulate core materials with a binder.

Embodiment 19: The method of Embodiment 18, wherein infiltrating the particulate core materials with a binder comprises placing a binder over the particulate core materials and heating the mold to melt the binder.

Embodiment 20: The method of Embodiment 19, wherein the strip comprises an organic binder and the binder comprises a metallic binder.

Embodiment 21: The method of Embodiment 3, wherein placing a template having a plurality of apertures over the substrate comprises placing a screen over the substrate.

Embodiment 22: The method of Embodiment 3, wherein placing at least some of the plurality of superabrasive particles at least partially within at least some of the apertures comprises causing at least some of the plurality of superabrasive particles to fall at least partially within the plurality of apertures in the screen by at least one of agitating, vibrating, blowing, and tilting.

Embodiment 23: The method of any of Embodiments 1 through 11, 21, or 22, further comprising forming the pattern by at least one of rapid prototyping, laser ablation, stamping, drilling, and cutting.

Embodiment 24: The method of any of Embodiments 1 through 11 or 21 through 23, further comprising mixing hard particles with a binder to form the strip.

Embodiment 25: The method of Embodiment 24, further comprising heating the strip to remove at least a substantial portion of the binder from the strip.

Embodiment 26: The method of any of Embodiments 1 through 11 or 21 through 25, further comprising sintering the strip and the superabrasive particles.

## 18

Embodiment 27: The method of Embodiment 7 or Embodiment 8, further comprising subjecting the strip, the superabrasive particles, and the another strip to a hot isostatic pressing process.

Embodiment 28: The method of any of Embodiments 7, 8, or 27, further comprising forming at least one of the material, the strip, and the another strip by at least one of rapid prototyping, laser ablation, stamping, drilling, and cutting.

Embodiment 29: The method of any of Embodiments 12 through 14, further comprising imparting the strip with a charge opposite the charge imparted to each of the plurality of superabrasive particles.

Embodiment 30: The method of any of Embodiments 12 through 14, further comprising electrically grounding the substrate before placing the plurality of charged superabrasive particles on the substrate.

Embodiment 31: The method of any of Embodiments 12 through 14, 29, or 30, wherein imparting like charges to each of a plurality of superabrasive particles comprises electrically charging the plurality of superabrasive particles with an electrostatic gun.

Embodiment 32: The method of any of Embodiments 12 through 14 or 29 through 31, wherein securing the superabrasive particles to the strip comprises forming a second strip over the superabrasive particles.

Embodiment 33: The method of Embodiment 9, wherein removing particles of the plurality that are not attracted to the adhesive comprises removing substantially all the particles except the particles attracted to the adhesive.

Embodiment 34: The method of Embodiment 9, wherein disposing a plurality of superabrasive particles over the strip comprises disposing one particle over each of a plurality of distinct areas of the adhesive.

Embodiment 35: The method of Embodiment 15 or Embodiment 16, further comprising bonding the second strip to the first strip and the third strip.

Embodiment 36: The method of any of Embodiments 15, 16, or 35, further comprising sintering the substrates and the superabrasive particles.

Embodiment 37: The method of Embodiment 18, further comprising preheating the strip to dissipate the first binder before placing particulate core materials in the mold.

Embodiment 38: The method of Embodiment 37, further comprising infiltrating the strip with a third binder before placing the strip in the mold.

Embodiment 39: The method of any of Embodiments 17 through 20, 37, or 38, further comprising infiltrating the strip with a metallic binder.

Embodiment 40: The method of any of Embodiments 17 through 20 or 37 through 39, wherein securing the insert to a body of the earth-boring rotary drill bit comprises attaching the substrate infiltrated with a metallic binder to an at least partially formed bit body by at least one of mechanical means, brazing, welding, and adhering.

Embodiment 41: An intermediate structure formed during the fabrication of an earth-boring tool, comprising a strip comprising a plurality of hard particles and a binder, a screen with a plurality of apertures therethrough placed over at least one surface of the strip, and a plurality of superabrasive particles. Each superabrasive particle of the plurality of superabrasive particles is disposed at least partially within an aperture of the plurality of apertures in the screen.

Embodiment 42: The intermediate structure of Embodiment 41, further comprising a plate disposed at least partially over the screen and the plurality of superabrasive particles,

19

the plate configured to press the plurality of superabrasive particles at least partially into the at least one surface of the strip.

Embodiment 43: The intermediate structure of Embodiment 41 or Embodiment 42, further comprising a roller disposed at least partially over the screen and the plurality of superabrasive particles for rolling over the plurality of superabrasive particles and pressing the plurality of superabrasive particles at least partially into the at least one surface of the strip.

Embodiment 44: The intermediate structure of any of Embodiments 41 through 43, wherein the plurality of hard particles of the strip comprises a plurality of tungsten carbide particles and the binder of the strip comprises an organic binder.

Embodiment 45: The intermediate structure of any of Embodiments 41 through 44, wherein the screen comprises wires.

Embodiment 46: The intermediate structure of any of Embodiments 41 through 44, wherein the screen comprises a metal plate.

Embodiment 47: The intermediate structure of any of Embodiments 41 through 46, wherein the screen with a plurality of apertures therethrough comprises a screen with a plurality of apertures arranged according to a predetermined pattern.

Embodiment 48: The intermediate structure of Embodiment 47, wherein the predetermined pattern of the apertures is at an angle to the direction of movement during operation of the earth-boring tool during normal operating conditions.

Embodiment 49: The intermediate structure of Embodiment 47 or Embodiment 48, wherein the predetermined pattern of the apertures is irregular, with a first concentration of apertures in one area of the screen and a second concentration of apertures in another area of the screen. The first and second concentrations different from each other.

Embodiment 50: The intermediate structure of any of Embodiments 41 through 44 or 49 through 49, wherein the plurality of apertures through the screen are formed by laser ablation.

Embodiment 51: An intermediate structure formed during the fabrication of an earth-boring tool, comprising a strip comprising a plurality of hard particles and a binder, and a plurality of electrically charged superabrasive particles at least partially covering at least one surface of the strip.

Embodiment 52: The intermediate structure of embodiment 51, wherein each electrically charged superabrasive particle of the plurality of electrically charged superabrasive particles comprises a coating of a chargeable material.

Embodiment 53: The intermediate structure of embodiment 52, wherein the coating of a chargeable material comprises tungsten.

Embodiment 54: The intermediate structure of any of Embodiments 51 through 53, wherein the strip is electrically grounded.

Embodiment 55: The intermediate structure of any of Embodiments 51 through 53, wherein the strip is electrically charged with a charge opposite to the charge of the plurality of superabrasive particles.

Embodiment 56: The intermediate structure of any of Embodiments 51 through 55, further comprising a plate over the charged superabrasive particles and the at least one surface of the strip for pressing the superabrasive particles at least partially into the at least one surface of the strip.

Embodiment 57: The intermediate structure of embodiment any of Embodiments 51 through 56, wherein the plu-

20

rality of electrically charged superabrasive particles comprises a plurality of diamonds.

Embodiment 58: A method of forming an insert for an earth-boring rotary drill bit, the method comprising forming a strip by mixing hard particles with a binder, arranging a plurality of superabrasive particles on a surface of the strip according to a predetermined pattern, and pressing the plurality of superabrasive particles at least partially into the surface of the strip.

10 Embodiment 59: The method of Embodiment 58, wherein arranging a plurality of superabrasive particles on a surface of the strip according to a predetermined pattern comprises placing a screen with a plurality of apertures arranged in a predetermined pattern over the strip, and placing a plurality of superabrasive particles over the screen such that at least some of the plurality of superabrasive particles are each disposed at least partially within each of at least some of the plurality of apertures in the screen.

15 Embodiment 60: The method of Embodiment 59, further comprising forming the plurality of apertures in the screen by at least one of laser ablation, stamping, drilling, and cutting.

20 Embodiment 61: The method of Embodiment 59 or Embodiment 60, further comprising causing the plurality of superabrasive particles to fall at least partially within the plurality of apertures in the screen by at least one of agitating, 25 vibrating, blowing, and tilting.

25 Embodiment 62: The method of any of Embodiments 58 through 61, wherein arranging a plurality of superabrasive particles on a surface of the strip according to a predetermined pattern comprises electrically charging the plurality of superabrasive particles, and placing the plurality of charged superabrasive particles on the strip.

30 Embodiment 63: The method of Embodiment 62, further comprising coating each superabrasive particle of the plurality of superabrasive particles with a chargeable material.

35 Embodiment 64: The method of Embodiment 62 or Embodiment 63, further comprising electrically charging the strip with a charge opposite that of the charged superabrasive particles.

40 Embodiment 65: The method of Embodiment 62 or Embodiment 63, further comprising electrically grounding the strip before placing the plurality of charged superabrasive particles on the strip.

45 Embodiment 66: The method of any of Embodiments 62 through 65, wherein electrically charging the plurality of superabrasive particles comprises electrically charging the plurality of superabrasive particles with an electrostatic gun.

50 Embodiment 67: The method of any of Embodiments 58 through 66, further comprising heating the strip to remove at least a substantial portion of the binder from the strip.

55 Embodiment 68: The method of any of Embodiments 58 through 66, further comprising infiltrating the strip with a metallic binder after arranging the plurality of superabrasive particles on a surface of the strip according to a predetermined pattern.

60 Embodiment 69: The method of any of Embodiments 58 through 68, wherein pressing the plurality of superabrasive particles at least partially into the surface of the strip comprises pressing the plurality of superabrasive particles at least partially into the surface of the strip with a metal plate.

65 Embodiment 70: The method of any of Embodiments 58 through 69, wherein pressing the plurality of superabrasive particles at least partially into the surface of the strip comprises pressing the plurality of superabrasive particles at least partially into the surface of the strip with a roller.

Embodiment 71: The method of any of Embodiments 58 through 70, wherein arranging a plurality of superabrasive

## 21

particles on a surface of the strip according to a predetermined pattern and pressing the plurality of superabrasive particles at least partially into the surface of the strip comprises arranging a plurality of diamonds on a surface of the strip according to a predetermined pattern and pressing the plurality of diamonds at least partially into the surface of the strip.

Embodiment 72: A method of forming an earth-boring rotary drill bit, comprising forming a strip by mixing hard particles with a first binder, pressing a plurality of superabrasive particles arranged in a predetermined pattern at least partially into the strip, forming the earth-boring rotary drill bit to include the strip after forming the strip, and pressing the plurality of superabrasive particles into the strip.

Embodiment 73: The method of Embodiment 72, wherein forming the earth-boring rotary drill bit comprises placing the strip in a mold for an earth-boring rotary drill bit, placing particulate core materials in the mold, and infiltrating the particulate core materials with a second binder.

Embodiment 74: The method of Embodiment 73, further comprising preheating the strip to dissipate the first binder before placing the particulate core materials in the mold.

Embodiment 75: The method of Embodiment 74, further comprising infiltrating the strip with a third binder before placing the strip in the mold.

Embodiment 76: The method of any of Embodiments 73 through 75, wherein infiltrating the particulate core materials with a second binder comprises placing a second binder over the particulate core materials and heating the mold to melt the second binder.

Embodiment 77: The method of any of Embodiments 73 through 76, wherein the first binder comprises an organic binder and the second binder comprises a metallic binder.

Embodiment 78: The method of any of Embodiments 72 through 77, further comprising infiltrating the strip with a metallic binder.

Embodiment 79: The method of any of Embodiments 72 through 78, wherein forming the earth-boring rotary drill bit to include the strip after forming the strip and pressing the plurality of superabrasive particles into the strip comprises attaching the strip infiltrated with a metallic binder to an at least partially formed bit body by at least one of mechanical means, brazing, welding, and adhering.

Embodiment 80: The method of Embodiment 1, further comprising selectively varying at least one of a diameter and a concentration of the superabrasive particles along a dimension of the insert for an earth-boring tool.

Embodiment 81: The method of Embodiment 80, further comprising selecting the dimension from the group consisting of a front-to-back dimension, a center-to-outside dimension, and a top-to-bottom dimension.

While the present invention has been described herein with respect to certain embodiments, those of ordinary skill in the art will recognize and appreciate that it is not so limited. Rather, many additions, deletions, and modifications to the embodiments depicted and described herein may be made without departing from the scope of the invention as herein-after claimed, and legal equivalents. In addition, features from one embodiment may be combined with features of another embodiment while still being encompassed within the scope of the invention as contemplated by the inventor. Further, embodiments of the disclosure have utility in drill bits having different bit profiles as well as different cutter types.

What is claimed is:

1. A method of forming an insert for an earth-boring tool, comprising:

## 22

forming a strip having a plurality of recesses therein, the strip configured to attract or secure a plurality of superabrasive particles;

after forming the strip having a plurality of recesses therein, disposing the plurality of superabrasive particles within the plurality of recesses;

securing at least some of the plurality of superabrasive particles within the recesses of the strip and forming an assembly including the strip having the plurality of recesses therein and the plurality of superabrasive particles secured within the recesses of the strip; and at least one of sintering the assembly, infiltrating the assembly with a metallic binder, and curing the assembly to form the insert for an earth-boring tool.

2. The method of claim 1, wherein securing at least some of the plurality of superabrasive particles within recesses of the strip comprises pressing at least some of the plurality of superabrasive particles into the strip.

3. The method of claim 1, wherein at least one of sintering the assembly, infiltrating the assembly with a metallic binder, and curing the assembly comprises infiltrating the assembly with a metallic binder after securing the plurality of superabrasive particles.

4. The method of claim 1, wherein disposing the plurality of superabrasive particles within the plurality of recesses comprises disposing a superabrasive particle within each recess of the plurality of recesses in the strip.

5. The method of claim 1, further comprising disposing another strip over the superabrasive particles and the strip to form a sandwiched array of superabrasive particles.

6. The method of claim 5, wherein disposing another strip over the superabrasive particles and the strip to form a sandwiched array of superabrasive particles comprises embedding at least some of the plurality of superabrasive particles into at least one of the strip and the another strip.

7. The method of claim 5, further comprising: disposing a superabrasive particle within each recess of a plurality of recesses of the another strip; and forming a third strip over the another strip and the superabrasive particles.

8. The method of claim 5, further comprising forming at least one of the strip and the another strip by rapid prototyping.

9. The method of claim 5, wherein disposing another strip over the superabrasive particles and the strip comprises aligning recesses of a lower surface of the another strip with the plurality of recesses of the strip.

10. The method of claim 1, further comprising coating each superabrasive particle of the plurality of superabrasive particles with a magnetic material and disposing a charged mesh under the strip.

11. The method of claim 1, further comprising selectively varying at least one of a diameter and a concentration of the superabrasive particles along a dimension of the insert for an earth-boring tool.

12. The method of claim 11, further comprising selecting the dimension from the group consisting of a front-to-back dimension, a center-to-outside dimension, and a top-to-bottom dimension.

13. A method of forming an insert for an earth-boring tool, comprising: coating each of a plurality of superabrasive particles with approximately 5 to 10 microns of a chargeable metal coating; imparting like charges to the plurality of superabrasive particles;

## 23

placing the plurality of superabrasive particles over a strip;  
and  
securing the plurality of superabrasive particles to the strip  
by one of charging conductive hard particles within the  
strip or electrically grounding the strip.

14. A method of forming an earth-boring rotary drill bit,  
comprising:

forming an insert, comprising:  
forming a strip having a plurality of recesses therein, the  
strip configured to attract or secure a plurality of  
superabrasive particles;  
after forming the strip having a plurality of recesses  
therein, disposing the plurality of superabrasive par-  
ticles within the plurality of recesses;  
securing at least some of the plurality of superabrasive  
particles within recesses of the strip and forming an  
assembly including the strip having the plurality of  
recess therein and the plurality of superabrasive par-  
ticles secured within the recesses of the strip; and

5

10

15

## 24

at least one of sintering the assembly, infiltrating the  
assembly with a metallic binder, and curing the  
assembly; and

securing the insert to a body of the earth-boring rotary drill  
bit.

15. The method of claim 14, wherein securing the insert to  
a body of the earth-boring rotary drill bit comprises:

placing the insert in a mold for an earth-boring rotary drill  
bit;

placing particulate core materials in the mold; and  
infiltrating the particulate core materials with a binder.

16. The method of claim 15, wherein the strip comprises an  
organic binder and the binder comprises a metallic binder.

17. The method of claim 13, wherein charging conductive  
hard particles within the strip comprises electrically charging  
the entire strip.

\* \* \* \* \*